

## UNITED STATES PATENT OFFICE

2,534,599

STABILIZED GELATINO SILVER HALIDE  
PHOTOGRAPHIC EMULSION

Dennis John Thomas Howe, Barnet, England, assignor to Elliott & Sons Limited, Barnet, England, a company of Great Britain

No Drawing. Application July 15, 1947, Serial No. 761,159. In Great Britain July 25, 1946

8 Claims. (Cl. 95—7)

1

This invention relates to compounds which serve as improvers and stabilizers for photographic gelatino silver halide emulsions.

In the production of photographic images in silver halide emulsions it is desirable that the maximum density of deposited silver should be as high as possible. This is especially the case when the photographic material is subjected to the process of hot glazing, where there is a tendency for the maximum density to be reduced and the image to assume a bronzed appearance. This is particularly noticeable in the case of emulsions composed principally of gelatino silver chloride.

Further, when a photographic emulsion is kept for some time, whether in the uncoated state or in the form of coated photographic material, its photographic properties tend to deteriorate, this deterioration being accelerated by humid and warm conditions. The most noticeable form of deterioration is the increase in fog value, particularly with the fast negative type of emulsion. The fog value of positive emulsions also has a tendency to increase on keeping, and with these emulsions continued keeping eventually leads to the production of images of poor colour, and to staining on extended development.

Compounds are known which, when added to an emulsion, will counteract one or other of these deficiencies. For instance, compounds are known which stabilize an emulsion against the increase of fog value. Among these are the organic compounds which form silver salts, the solubility of which at 18° C. does not surpass that of silver chloride. A specific compound of this type is the mono mercapto triazole, n-ethyl thiotriazole. But while they may be effective as stabilizers these and other compounds cause a serious reduction in speed of the photographic emulsion in which they are applied.

In accordance with the present invention it has been found that the deterioration of the emulsion due to ageing can be reduced, particularly with regard to increase in fog value, and in addition the quality of the image and the maximum density, particularly after hot glazing, can be improved, by the use of a substituted dithiourazole.

According to one form of the present invention, therefore, a gelatino silver halide emulsion may be improved with regard to stabilization for the formation of fog by adding to the material, at any stage, not later than development, a small quantity of a substituted dithiourazole.

The substituted dithiourazoles which are of

2

use as improvers or stabilizers have the general molecular formula:



10 where R<sub>1</sub> and R<sub>2</sub> are either hydrogen or alkyl, aryl or aralkyl molecular groups but are not both hydrogen. This formula is shown in the keto form, but all tautomeric forms are included in the scope of the invention. The dienol form may also be named 3,5-dimercapto 1,2,4 triazole.

15 Examples of compounds having this general formula are:

- 1 phenyl dithiourazole,  
4 phenyl dithiourazole,  
20 4 methyl dithiourazole,  
1 ethyl dithiourazole.

25 4 substituted dithiourazoles may be prepared by treating the corresponding substituted hydrazo dithiocarbonamide with hydrochloric acid or caustic soda solution as described in "Berichte der Deutschen Chemischen Gesellschaft," 1922, vol. 1, page 352 (55th year).

The preparation of 1 phenyl dithiourazole is described in "Berichte der Deutschen Chemischen Gesellschaft," 1904, vol. 1, page 184 (37th year).

30 The substituted dithiourazoles or dithiourazole compounds as described above give rise to a smaller reduction in speed than do compounds hitherto proposed for similar purposes.

35 Gelatino silver chloride emulsions containing a dithiourazole compound are capable of producing a higher maximum black after hot glazing than does such an emulsion containing one of the compounds previously proposed for this purpose, for example, a mono mercapto triazole. While this invention is independent of any particular theory it is suggested that this is possibly due to the presence of two potential reactive groups in the dithiourazole compound compared 40 with the one reactive group in the previously proposed compounds.

The dithiourazole compound may be incorporated in the emulsion as an addition, conveniently in the form of a solution of the free substance 45 or one of its salts, during or subsequent to the preparation of the emulsion. Other methods of bringing the compound in operative contact with the emulsion may be used such as including it in the subcoat, supercoat, backing layer, a filter layer, or in the wrapping material.

As mentioned above the dithiourazole compounds do not cause so great a reduction in speed as that which results from the use of some of the other compounds hitherto proposed. This is particularly the case with certain substituted dithiourazoles such as the 1 or 4 phenyl dithiourazole where the quantity required for use as an improver has a practically negligible effect on speed and contrast. However, when used in the free state, certain other dithiourazole compounds, may cause a slight alteration in the photographic properties of the emulsion. To minimise any such alteration of properties the addition should preferably be made after the final digestion period rather than at an earlier stage of emulsion manufacture. If stabilization against fog is the improvement required, then obviously the dithiourazole compound must be in operative contact with the emulsion during keeping and before development.

Naturally, it is an advantage for the manufacturer to be able to incorporate the dithiourazole compounds in the photographic material, and should he wish to use a dithiourazole compound which in its free state would have an adverse effect on the emulsion, this may be accomplished without this adverse effect by using it in the form of a metal salt which is substantially water insoluble but decomposable by treatment of the photographic element in a processing bath subsequent to development. The silver salt of a dithiourazole compound is most useful when added to the emulsion or to a layer in contact with the emulsion. Other metal salts may be used, including thallous, ferric, and copper salts.

It is advisable for the metal salt to be in a fine state of subdivision in the layer in which it is incorporated. A convenient method of achieving this is to deposit the metal salt in situ in the colloidal medium in which it is dispersed, by the double decomposition of a water soluble metal salt and a water soluble salt of the dithiourazole compound in gelatine solution.

The quantity of the dithiourazole compound or its soluble salt employed varies with the purpose for which it is used, and with the method adopted for bringing it into operative contact with the emulsion. For direct addition, from 1 cc. to 40 cc. of  $1/1000$  solution per litre of emulsion is suitable if the improvement required is stabilization, particularly of a fast negative emulsion, and it is advisable to select a compound for use which has little or no detrimental effect on the properties of the emulsion such, for example, as an aryl substituted dithiourazole.

To improve the maximum density of image produced in a positive emulsion the quantity suitable for a litre of emulsion is from 1 cc. to 70 cc. of  $1/1000$  solution. The solution may be in water or in a water miscible organic solvent which does not have a detrimental effect on the emulsion. If the additions are made to colloids which are to be coated adjacent to the emulsion layer, then higher quantities are preferable, approximately twice the quantity that would be used for a similar quantity of emulsion being required. These quantities are not given to limit the invention but merely as an indication of the order of the quantity of the compound to be used to give the best results.

Usually smaller quantities give less marked improvements, while higher quantities produce no additional improvement and moreover tend to affect the photographic properties adversely to a greater extent.

However, with the nonsoluble salts of the dithiourazole compounds, much greater quantities may be used without detriment to the photographic properties, whether the salts are included in the emulsion or in adjacent layers.

The following examples illustrate the invention, but it will be appreciated that invention is not limited to the specific materials, quantities, methods or other features described therein.

#### Example 1

Three separate 1-lb. quantities of a negative gelatino silver iodo bromide emulsion having a silver content equivalent to 20 gms. silver nitrate per 1-lb. of emulsion were taken and panchromatized. To one part was added the normal coating additions and it was coated on to glass plates (material A). The second quantity was coated after 13 cc. of  $1/1000$  spirit solution of 4 phenyl 3.5 dithiourazole had been added (material B). The third quantity was coated after 13 cc. of  $1/1000$  spirit solution of 1 phenyl 3.5 dithiourazole had been similarly added (material C).

Fresh coated test portions of the material were exposed behind a density step wedge and processed, and the fog values of materials A, B and C were determined. Other test portions were kept at 110° F. and at a relative humidity of 70% for two weeks. These materials were similarly tested and the fog values determined. The fog values were as follows:

| Material | Freshly coated | After two weeks incubation |
|----------|----------------|----------------------------|
| A        | 0.13           | 0.24                       |
| B        | 0.11           | 0.14                       |
| C        | 0.13           | 0.15                       |

#### Example 2

3-lbs. of a gelatino silver bromide positive ("Bromide") emulsion were divided equally. One half was coated on to paper normally (material A), and the other half was likewise coated after addition of 20 cc. of  $1/1000$  aqueous solution of 1 phenyl 3.5 dithiourazole had been made to it (material D). When dry test samples of each of the coated materials were exposed behind a density step wedge, developed, fixed and glazed on a commercial hot glazing machine. Maximum density and speed were determined for each material. A sample of each material was incubated for two weeks at 110° F. at a relative humidity of 70% and the condition of material noted after development for 6 minutes in a standard MQ developer, at 18° C. with the following results:

| Material | Maximum density on hot glazing | Condition of incubated sample on forced development |
|----------|--------------------------------|-----------------------------------------------------|
| A        | 1.78                           | Stained.                                            |
| D        | 1.92                           | No stain.                                           |

There was no appreciable difference in speed and contrast between materials A and D.

#### Example 3

1½-lbs. of gelatino silver chloride emulsion were coated in the normal manner on to paper (material A). To another 1½-lbs. of the same emulsion were added 12 cc. of  $1/1000$  spirit solution of 4 phenyl 3.5 dithiourazole and the emulsion



## REFERENCES CITED

The following references are of record in the file of this patent:

## UNITED STATES PATENTS

| Number    | Name     | Date             |
|-----------|----------|------------------|
| 1,560,240 | Jelley   | Nov. 3, 1925     |
| 2,066,099 | Dieterle | Dec. 29, 1936    |
| 2,353,754 | Peterson | July 18, 1944    |
| 2,432,506 | Chilton  | Dec. 16, 1947 10 |

Number

163,039  
436,576

5

## FOREIGN PATENTS

| Country       | Date           |
|---------------|----------------|
| Switzerland   | Sept. 16, 1933 |
| Great Britain | Jan. 6, 1934   |

## OTHER REFERENCES

Berichte der deutschen Chem. Ges., 1895, vol. I, page 949; ibid., 1922, vol. I, page 352; ibid., 1904, vol. I, page 184.